# EUROPEAN PATENT SPECIFICATION

(11) **EP 0 293 961 B1**
(45) Date of publication and mention of the grant of the patent: **14.08.1991**
(21) Application number: 88200895.6
(22) Date of filing: 06.05.1988
(51) Int. Cl.: B22D 27/13, B22D 27/08

(54) **Casting method and apparatus therefor**
Giessverfahren und Vorrichtung dazu
Procédé et dispositif pour la coulée

(30) Priority: 30.05.1987 GB 8712743
(43) Date of publication of application: 07.12.1988
(73) Proprietor: AE PLC, Rugby Warwickshire CV22 7SB (GB)
(72) Inventor: Paine, Brian, Bradford West Yorkshire BD2 3SE (GB)
(74) Representative: Goddard, David John

(56) References cited:
- DE-A- 3 220 744
- DE-A- 3 603 310
- FR-A- 2 255 983
- GB-A- 1 356 890
- GB-A- 1 472 288
- US-A- 3 568 752

## Description

The present invention relates to a method and apparatus for casting of articles according to the preambles of claims 1 and 10, respectively.

Such a method and such an apparatus are known from GB-A-1356890.

In our co-pending patent application 0293960 of even filing date herewith and claiming priority from British patent application No 8712742 filed on 30 May 1987, a method and apparatus are described for the production of cast components having an equiaxed grain structure and reduced levels of shrinkage porosity.

The method comprises casting molten metal into a mould under reduced pressure or under a protective atmosphere in a first chamber and then immediately withdrawing the filled mould containing the molten metal into a second chamber and increasing the pressure in the second chamber with a fluid up to a maximum pressure of 7 MPa until at least partial solidification has occurred. Apparatus is also described for carrying out the method of the invention.

The method and apparatus described in co-pending EP 0293960 is particularly suitable for gas turbine engine components such as blades and nozzle guide vanes, for example, which are cast in gas permeable ceramic moulds. Such components as blades, for example, possess substantial differences in section between the root and airfoil portions which leads, in conventional casting methods for components having equiaxed grain structures, to shrinkage porosity in the thinner airfoil portion.

The method described in co-pending EP 0293960 ensures enhanced feeding of liquid metal to solidifying regions by pressurisation and thus producing reduced levels of porosity.

There is a need, however, to produce components which have very considerable differences in section.

Such components include turbine wheels for gas turbine engines and turbochargers, for example, where a multiplicity of airfoils are cast integrally with a hub or disc portion.

In such components there is not only a problem with porosity in the thinner airfoil portions but there is an additional problem with the grain structure in the hub portion. Because of the generally thick and relatively extensive section of the hub portion large columnar grains tend to grow unchecked. Such grain structures are detrimental to the mechanical properties of the hub which needs to be able to withstand very high forces during operation. An equiaxed grain structure in the hub is highly desirable. It is known to prevent the formation of columnar grains by oscillating the filled mould about an axis eccentric to the component axis. Such oscillation causes mass movement within the solidifying mushy metal and breaks up the growing metal dendrites before they become too large and firmly set as growing columnar grains. A generally equiaxed grain structure is thus produced.

The method and apparatus of the present invention provide components which have large section differences with both an equiaxed grain structure and reduced levels of porosity.

According to a first aspect of the present invention there is provided a method for the production of cast components. The method comprises the steps of heating a mould, filling the mould with molten metal in a first chamber, withdrawing the filled mould into a second chamber, isolating the second chamber from the first chamber with regard to pressure, characterised by pressurising the second chamber with a gas up to a maximum pressure of 7 MPa and oscillating the filled mould whilst under pressure until at least partial solidification has occurred.

In the case of turbine components cast from iron-, nickel- or cobalt-based superalloys the metal may be cast in the first chamber under reduced pressure or under a protective atmosphere.

Heating of the mould in the first chamber rather than solely preheating in an external preheating furnace provides greater control and flexibility of preheating and is obtainable by means of, for example, radiant heaters.

Preferably, the pressurising gas has little or no chemical reaction with the molten metal. Examples may include argon, helium and nitrogen.

Preferably the pressure may be applied to the filled mould in the mould chamber within 60 seconds of the completion of pouring and more preferably within 30 seconds.

The mould may be oscillated about an axis which is eccentric to the axis of the component being cast.

The mould may be oscillated within a frequency range of from 5 to 500 cycles per minute.

The amplitude of oscillation may lie in the range from 5° to 360° in any one cycle or may be in excess of one complete revolution of the mould.

Frequency and amplitude of oscillation will vary with component dimensions and geometry and furthermore may also vary during the solidification process itself and be affected by the alloy being cast.

According to a second aspect of the present invention there is provided apparatus for the production of cast components. The apparatus comprises a casting chamber, metal melting and pouring means, mould heating means, a mould chamber adjacent the casting chamber and connected thereto by valve means of sufficient size to allow a mould to pass therethrough, mould moving means to move the mould between the casting chamber and the mould chamber characterised by having pressurising means for pressurising the mould chamber with a gas and means for oscillating the mould in the mould chamber whilst under pressure.

The casting chamber may also have vacuum pump means associated with it, as may the mould chamber, for producing a reduced pressure within the chambers.

Alternatively or additionally the chambers may be provided with suitable connections for producing a gaseous protective atmosphere such as with argon, for example, within the chambers.

In order that the present invention may be more fully understood an example will now be described by way of illustration only with reference to the accompanying drawings, of which:
Figure 1 shows a schematic section through apparatus according to the present invention prior to casting metal into the mould;
Figure 2 shows part of the apparatus of Figure 1 after casting; and
Figure 3 which shows a section through an alternative construction of apparatus for oscillating the mould.

Referring now to Figures 1 and 2 and where the same features are denoted by common reference numerals. The apparatus is shown generally at 10 and comprises a vacuum casting chamber 11 which includes a port 12 connected to a vacuum pump (not shown). Contained in the chamber 11 is a coil box assembly 13 having induction heating coils (not shown) and crucible 14; the assembly 13 being mounted such that it may be tilted to pour the molten metal 15 in known manner. The chamber also includes a port 16 and vacuum lock 17 to enable the crucible 14 to be recharged with fresh metal whilst under vacuum. In the bottom wall 20 of the chamber 11 is an aperture 21 of sufficient size to allow a mould assembly 22, having an axis 22a, to pass therethrough. Above and surrounding the aperture 21 is a mould heating chamber 23 which comprises an outer insulating box 24 having contained therein known radiant heating means 25 having the appropriate power supply and control means (not shown) attached thereto. In the top of the insulation box 24 is an aperture having a pouring tube 27 therein to guide the molten metal into the mould 22 on pouring. Below the vacuum chamber 11 is a mould chamber 30. The mould chamber 30 is attached in sealed engagement to the bottom wall 20 of the casting chamber 11. The chamber 30 may be isolated from the chamber 11 by means of the isolation valve 31 and seal 32. The valve 31 may be moved between the open position (Figure 1) and the closed position (Figure 2) by suitable known remotely operated control means (not shown). Cooling passages 33 are provided around the chamber wall. The chamber 30 has a door 34 in the wall to allow positioning and subsequent removal of the mould 22, the door 34 is sealable to the chamber wall 35. Also provided in the chamber wall 35 is a vacuum pumping port 36 connected to a vacuum pump (not shown) via a valve 37. A further port 38 in the wall 35 is provided to supply fluid under pressure from a fluid supply source (not shown) via a valve 39. The mould 22 is mounted on a table 40 but insulated therefrom by an insulation block 41. The table 40 is itself mounted on a movable ram 42 having an axis 43 and which ram may slide in sealed engagement with the bottom wall 45 of the chamber 30 and also rotate or oscillate in sealed engagement therewith. A bearing 46 in the bottom wall 45 supports the ram in both sliding and oscillatory movement. The ram 42 also includes passages 48 for provision of coolant. At the lower end of the ram 42 is a second bearing 49 and a manifold 50 to connect coolant pipes 51, 52 to the ram and allow oscillatory movement. A pulley wheel 54 is mounted on the lower end of the ram 42 and which pulley wheel is drivably connected to a second pulley wheel 55 by a transmission belt 56. The pulley wheel 55 is driven by an electric motor 58 which has appropriate power supplies (not shown) and control means (not shown). The motor 58 and bearing 49 are both mounted on a platform 60 which is itself mounted on a ram 61. The platform 60 may be varied in height relative to the bottom wall 45 of the chamber 30.

In operation the chamber 11 is pumped down to a pressure appropriate to the requirements of the alloy being cast. The valve 31 is closed against the seal 32 and the ram retracted to its position within the chamber 30. The mould 22 is placed and secured on the insulation block 41, the door 34 closed and sealed and the chamber 30 pumped down to a pressure in the region of that in chamber 11. The valve 31 is opened and the ram 42 elevated to move the mould 22 into the mould heating chamber 23. The mould is heated by the radiant heaters 25 to a desired temperature and once at the desired temperature molten metal 15 at a a second desired temperature is poured from the assembly 13 into the mould 33 via the pouring tube 27. The filled mould is immediately withdrawn from the chamber 23 into the chamber 30 and the valve 31 is closed against the seal 32 whereupon the valve 37 is closed and the valve 39 opened to pressurise the chamber 30 with fluid such as argon for example. The pressure may be brought to bear against the molten metal in a time of less than 20 seconds and may be raised to a maximum pressure of about 7 MPa. The filled mould 22 is now oscillated about the ram axis 43 at a frequency of 280 cycles/min. and an amplitude of 70°. Since the axis 22a of the mould is eccentric to the axis 43 the metal in the mould in the thicker sections, and which comprises a mixture of liquid metal and growing metal dendrites, is aggitated and causes the growing dendrites to be broken up thus preventing the formation of undesirable, coarse columnar grains. The pressure within the chamber 30 assists in the feeding of liquid metal to the solidifying portions to eliminate or minimise the formation of shrinkage porosity. Oscillation frequency and amplitude may be varied during the course of solidification and may only be applied for part of the time required to achieve complete solidification. Similarly the pressure may be released before complete solidification has occurred.

Figure 3 shows an alternative construction of drive for oscillating the mould 22. In this construction the ram 42 does not itself oscillate. Interposed between the ram table 40 and the insulation block 41 is a carrier 70 which is free to rotate on the table 40 supported by a rolling element bearing 71. On the outer periphery of the carier 70 is a gear toothed ring 72 which, when the ram 42 is lowered to its lowermost extent, meshes with a gear pinion 73 driven by an electric motor 74. The motor 74 is connected to suitable control apparatus (not shown) situated outside the chamber 30.

In the examples given above the article being cast is a turbine disc and blade unit having rotational symmetry. Such symmetry is not necessary as any article which has widely different section thicknesses included therein may be cast by the method and apparatus of the present invention.

Many modifications may be made to the embodiment shown. Such modifications may relate to the type of valve employed to seal the casting chamber from the mould chamber and to the method and precise apparatus used to move the ram and mould between chambers and also the means used to oscillate the mould.

The ram 42 may be elevated by electrical or hydraulic means, for example.

## Claims

1. A method for the production of cast components, the method comprising the steps of heating a mould (22), filling the mould with molten metal in a first chamber (11), withdrawing the filled mould into a second chamber (30), isolating the second chamber from the first chamber with regard to pressure characterised by pressurising the second chamber with a gas up to a maximum pressure of 7 MPa and oscillating the filled mould whilst under pressure until at least partial solidification has occurred.

2. A method according to claim 1 characterised in that the filled mould is oscillated within a frequency range of 5 to 500 cycles per minute.

3. A method according to either claim 1 or claim 2 characterised in that the amplitude of oscillation is greater than one complete revolution.

4. A method according to either claim 1 or claim 2 characterised in that the amplitude of oscillation lies in the range of 5° to 360°.

5. A method according to any one preceding claim characterised in that the gas is selected from the group comprising helium, argon and nitrogen.

6. A method according to any one preceding claim characterised in that the mould is oscillated about an axis which is eccentric to the axis of the component being cast.

7. A method according to any one preceding claim characterised in that the pressure is applied within 60 seconds of the completion of pouring of the molten metal.

8. A method according to claim 7 characterised in that the pressure is applied within 30 seconds of pouring.

9. A method according to any one preceding claim characterised in that the metal being cast is selected from the group comprising aluminium alloys, copper alloys, iron alloys, nickel alloys and cobalt alloys.

10. Apparatus for the production of cast components, the apparatus comprising a casting chamber (11), metal melting and pouring means (13), mould heating means (23), a mould chamber (30) adjacent the casting chamber and connected thereto by valve means (21, 31) of sufficient size to allow a mould (22) to pass therethrough, mould moving means (42) to move the mould between the casting chamber and the mould chamber characterised by having pressurising means (38, 39) for pressurising the mould chamber with a gas and means (54, 55, 56, 58) for oscillating the mould in the mould chamber whilst under pressure.

11. Apparatus according to claim 10 characterised in that the mould axis (22a) and the axis of oscillation (43) are not coincident.

12. Apparatus according to either claim 10 or claim 11 characterised in that the casting chamber and the mould chamber are provided with vacuum pumping means.

13. Apparatus according to any one of claims 10 to 12 characterised in that the mould moving means comprises a height positionable ram which is itself oscillatable about its axis.

## Revendications

1. Procédé pour la production de composants coulés, comprenant les étapes consistant à chauffer un moule (22), à remplir le moule de métal fondu dans une première chambre (11), à retirer le moule plein pour le mettre dans une seconde chambre (30), et à isoler la seconde chambre de la première chambre en ce qui concerne la pression, caractérisé par la mise sous pression de la seconde chambre au moyen d'un gaz jusqu'à une pression maximale de 7 MPa et la soumission à des oscillations du moule plein et soumis à la pression jusqu'à ce qu'une solidification partielle au moins ait eu lieu.

2. Procédé selon la revendication 1, caractérisé en ce qu'on fait osciller le moule rempli dans les limites d'une plage de fréquences de 5 à 500 cycles à la minute.

3. Procédé selon la revendication 1 ou la revendication 2, caractérisé en ce que l'amplitude des oscillations est supérieure à un tour complet.

4. Procédé selon la revendication 1 ou la revendication 2, caractérisé en ce que l'amplitude des oscillations est située dans la plage comprise entre 5° et 360°.

5. Procédé selon l'une quelconque des revendications précédentes, caractérisé en ce que le gaz est choisi dans le groupe comprenant l'hélium, l'argon et l'azote.

6. Procédé selon l'une quelconque des revendications précédentes, caractérisé en ce que l'on fait osciller le moule autour d'un axe qui est excentrique par rapport à l'axe du composant qui est coulé.

7. Procédé selon l'une quelconque des revendications précédentes, caractérisé en ce que la pression est appliquée dans les 60 secondes après la fin du versage du métal fondu.

8. Procédé selon la revendication 7, caractérisé en ce que la pression est appliquée dans les 30 secondes après le versage.

9. Procédé selon l'une quelconque des revendications précédentes, caractérisé en ce que le métal qui est fondu est choisi dans le groupe comprenant des alliages d'aluminium, des alliages de cuivre, des alliages de fer, des alliages de nickel et des alliages de cobalt.

10. Dispositif pour la production de composants coulés, comprenant une chambre de coulée (11), des moyens (13) de mise en fusion et de versage du métal, des moyens (23) de chauffage du moule, une chambre de moulage (30) adjacente à la chambre de coulée et reliée à celle-ci par des moyens à vanne (21, 31) de dimensions suffisantes pour permettre au moule (22) d'y passer, et des moyens de déplacement de moule (42) pour déplacer le moule entre la chambre de coulée et la chambre de moulage, caractérisé en ce qu'il comprend des moyens de pressurisation (38, 39) pour pressuriser la chambre de moulage avec un gaz et des moyens (54, 55, 56, 58) pour faire osciller le moule dans la seconde chambre alors qu'il est sous pression.

11. Dispositif selon la revendication 10, caractérisé en ce que l'axe (22a) du moule et l'axe d'oscillation (43) ne coïncident pas.

12. Dispositif selon la revendication 10 ou 11, caractérisé en ce que la chambre de coulée et la chambre de moulage sont munies de moyens de pompage de vide.

13. Dispositif selon l'une quelconque des revendications 10 à 12, caractérisé en ce que les moyens de déplacement du moule comprennent un vérin pouvant être positionné en hauteur et pouvant osciller autour de son axe.

## Patentansprüche

1. Verfahren zur Herstellung von Gußteilen, das die Schritte des Aufheizens einer Form (22), des Füllens der Form mit Metallschmelze in einer ersten Kammer (11), des Zurückfahrens der gefüllten Form in eine zweite Kammer (30) und des Druckisolierens der zweiten Kammer gegenüber der ersten Kammer umfaßt, **dadurch gekennzeichnet**, daß die zweite Kammer mit einem Gas bis zu einem maximalen Druck von 7 MPa unter Druck gesetzt und die gefüllte Form, während sie unter Druck steht, in Schwingungen versetzt wird, bis zumindest eine teilweise Erstarrung eingetreten ist.

2. Verfahren nach Anspruch 1, dadurch gekennzeichnet, daß die gefüllte Form in Schwingungen innerhalb eines Frequenzbereiches von 5 bis 500 Zyklen pro Minute versetzt wird.

3. Verfahren nach Anspruch 1 oder 2, dadurch gekennzeichnet, daß die Schwingungsamplitude größer als eine volle Umdrehung ist.

4. verfahren nach Anspruch 1 oder 2, dadurch gekennzeichnet, daß die Schwingungsamplitude im Bereich von 5° bis 360° liegt.

5. Verfahren nach einem der vorhergehenden Ansprüche, dadurch gekennzeichnet, daß das Gas aus der Gruppe ausgewählt wird, die Helium, Argon und Stickstoff umfaßt.

6. Verfahren nach einem der vorhergehenden Ansprüche, dadurch gekennzeichnet, daß die Form um eine Achse, die exzentrisch zur Achse des zu gießenden Teiles liegt, in Schwingungen versetzt wird.

7. Verfahren nach einem der vorhergehenden Ansprüche, dadurch gekennzeichnet, daß der Druck innerhalb von 60 Sekunden nach Beendigung des Eingießens der Metallschmelze aufgebracht wird.

8. Verfahren nach Anspruch 7, dadurch gekennzeichnet, daß der Druck innerhalb von 30 Sekunden nach dem Eingießen aufgebracht wird.

9. Verfahren nach einem der vorhergehenden Ansprüche, dadurch gekennzeichnet, daß das zu vergießende Metall aus der Gruppe ausgewählt wird, die Aluminiumlegierungen, Kupferlegierungen, Eisenlegierungen, Nickellegierungen und Kobaltlegierungen umfaßt.

10. Vorrichtung zur Herstellung von Gußteilen, mit einer Gießkammer (11), einer Einrichtung (13) zum Schmelzen und Vergießen des Metalls, einer Einrichtung (23) zum Erhitzen einer Farm, einer Formkammer (30), die der Gießkammer Benachbart und mit dieser über Ventile (21, 31) ausreichender Größe zum Durchlaß einer Form (22) verbunden ist, und mit einer Einrichtung (42) zum Verfahren der Form zwischen der Gießkammer und der Formkammer, **gekennzeichnet** durch eine Druckerzeugungseinrichtung (38, 39), um die Formkammer mit einem Gas unter Druck zu setzen, und durch eine Einrichtung (54, 55, 56, 58), mit der die Form in der Formkammer in Schwingungen versetzbar ist, während sie unter Druck gehalten wird.

11. Vorrichtung nach Anspruch 10, dadurch gekennzeichnet, daß die Formachse (22a) und die Schwingungsachse (43) nicht zusammenfallen.

12. Vorrichtung nach Anspruch 10 oder 11, dadurch gekennzeichnet, daß die Gießkammer und die Formkammer mit Vakuumpumpeinrichtungen versehen sind.

13. Vorrichtung nach einem der Ansprüche 10 bis 12, dadurch gekennzeichnet, daß die Einrichtung zum Verfahren der Form einen höhenverstellbaren Stab aufweist, der selbst um seine Achse verschwingbar ist.
